

# UNITED STATES PATENT OFFICE.

IGNATZ KREIDL, OF VIENNA, AUSTRIA-HUNGARY.

## LOADED SILK AND PROCESS OF LOADING THE SILK.

1,173,196.

Specification of Letters Patent. Patented Feb. 29, 1916.

No Drawing.

Application filed May 27, 1910. Serial No. 563,776.

To all whom it may concern:

Be it known that I, IGNATZ KREIDL, chemist-manufacturer, a subject of the Emperor of Austria-Hungary, and a resident of XXI/1 Kohlgasse 7, Vienna, in the Empire of Austria-Hungary, have invented Improvements in Loaded Silk and Process of Loading the Silk; and I do hereby declare the following to be a full, clear, and exact 10 description of the invention, such as will enable others skilled in the art to which it appertains to make and use the same.

This invention relates to the loading of silk.

It has hitherto been the practice to load silk by saturating it with metallic salt solutions, preferably chlorid of tin solutions, and then to wash it. The metallic salt fixed on the fiber and which, as such is chiefly 15 harmful on account of its acidity, is then transformed into the less harmful phosphate by sodium phosphate. The salts formed during the transformation must be completely washed out, as their presence is harmful 20 to the silk and might possibly render it useless. The washing is a protracted operation, as it has to be repeated several 25 times and is detrimental to the strength and elasticity of the silk.

The object of the present invention is to provide a process for the loading of silk wherein the formation or use of injurious salts is avoided, to provide a simplified process and one wherein a superior product 30 is obtained. According to the present invention, this is achieved by the use of colloidal metallic hydrates ("sol") in solution, for instance, water solution, and more particularly those of zirconium and other rare 35 earth metals or mixtures of such solutions, in place of the metallic salt solutions.

Examples of hydrates of rare earth metals other than zirconium which may be used are those of the metals of the groups of the 40 cerite and ytterite earths, and of the group of the thorium earths, particularly the salts of the representatives of these groups which are found in Group IV of the periodic arrangement. Cerium hydrate is however 45 preferably not employed alone, but mixed with other hydrates. These hydrates have in common a high atomic weight and a strong tendency to colloidal formation. These solutions, in which the electrolyte 50 possibly still adhering is only present in very small quantities, offer the advantage

that they act directly as a loading medium, as they are very thoroughly absorbed by the fiber and fixed, and owing to their neutrality do not attack the fiber. As the transformation hitherto required is not necessary and their presence does not harm the fiber, the repeated washing is unnecessary and may be dispensed with.

If a particularly good fixing of the colloidal metallic hydrate on the fiber is desired, the dissolved "sol" on the fiber may also be formed into the insoluble form called "gel" by any coagulating medium, for which purpose only small quantities of 60 65 70 the coagulating medium need be used.

A subsequent treatment such as washing can be dispensed with in this process, as bodies which are not harmful to the silk may be used as coagulating media.

In carrying the loading process into effect the silk is dipped into a bath consisting of a colloidal metallic hydrate solution, preferably of zirconium. The concentration of the bath depends upon the degree of loading desired, and the fixing of the colloidal metallic hydrate on the fiber takes place in the bath. The dipping and therefore the fixing of the colloidal metallic hydrate is 75 80 85 repeated until the desired loading is obtained.

That part of the metallic hydrate solution not absorbed by the fiber can either be washed out with water or simultaneously transformed into "gel" and fixed on the 90 fiber with the absorbed "sol" by a coagulating medium, e. g. sodium phosphate.

What I claim as my invention and desire to secure by Letters Patent is:

1. In the loading of silk, the process which 95 consists in saturating the silk with a colloidal metallic hydrate solution, the hydrate being one which is readily absorbed by the silk, and which does not readily attack the silk, and the metal constituent having a 100 high atomic weight.

2. In the loading of silk, the process which 105 consists in saturating the silk with a solution of mixed colloidal metallic hydrates, the hydrates being those which are readily absorbed by the silk, and which do not readily attack the silk, and the metal constituent having a high atomic weight.

3. In the loading of silk, the process which 110 consists in saturating the silk with a colloidal hydrate solution of a rare earth metal, the hydrate being one which is readily ab-

sorbed by the silk, and which does not readily attack the silk, and the metal constituent having a high atomic weight.

4. In the loading of silk, the process which 5 consists in saturating the silk with a solution of mixed colloidal hydrates of the rare earth metals, the hydrates being those which are readily absorbed by the silk, and which do not readily attack the silk, and the metal 10 constituent having a high atomic weight.

5. In the loading of silk, the process which consists in saturating the silk with a colloidal solution of zirconium hydrate.

6. In the loading of silk, the process which 15 consists in saturating the silk with a colloidal metallic hydrate solution and transforming the "sol" into "gel", the hydrate being one which is readily absorbed by the silk, and which does not readily attack the 20 silk, and the metal constituent having a high atomic weight.

7. In the loading of silk, the process which consists in saturating the silk with a solution of mixed colloidal metallic hydrates 25 and transforming the "sol" into "gel", the hydrates being those which are readily absorbed by the silk, and which do not readily attack the silk, and the metal constituent having a high atomic weight.

30 8. In the loading of silk, the process which consists in saturating the silk with a colloidal hydrate solution of a rare earth metal and transforming the "sol" into "gel"; the hydrate being one which is readily absorbed by the silk, and which does not readily attack the silk, and the metal constituent having a high atomic weight.

9. In the loading of silk, the process which 35 consists in saturating the silk with a solution of mixed colloidal hydrates of the rare earth metals, and transforming "sol" into "gel", the hydrates being those which are readily absorbed by the silk, and which do

not readily attack the silk, and the metal constituent having a high atomic weight. 45

10. In the loading of silk, the process which consists in saturating the silk with a colloidal hydrate solution of zirconium and transforming the "sol" into "gel".

11. As a new article of manufacture, silk 50 loaded with a colloidal hydrate of a rare earth metal, the hydrate being one which is readily absorbed by the silk, and which does not readily attack the silk, and the metal constituent having a high atomic weight. 55

12. As a new article of manufacture, silk loaded with colloidal metallic hydrate in the form of "gel", the hydrate being one which is readily absorbed by the silk, and which does not readily attack the silk, and the metal constituent having a high atomic weight. 60

13. As a new article of manufacture, silk loaded with a mixture of colloidal hydrates of the rare earth metals, the hydrates being 65 those which are readily absorbed by the silk, and which do not readily attack the silk, and the metal constituent having a high atomic weight.

14. As a new article of manufacture, silk 70 loaded with a colloidal hydrate of zirconium.

15. As a new article of manufacture, silk loaded with a colloidal metallic hydrate of a rare earth metal in the form of "gel", the 75 hydrate being one which is readily absorbed by the silk, and which does not readily attack the silk, and the metal constituent having a high atomic weight.

16. As a new article of manufacture, silk 80 loaded with a colloidal hydrate of zirconium in the form of a "gel".

In testimony whereof I have signed my name to this specification.

DR. IGNATZ KREIDL.

Copies of this patent may be obtained for five cents each, by addressing the "Commissioner of Patents.  
Washington, D. C."